

# UNITED STATES PATENT OFFICE.

LUTHER B. LOCKHART, OF ATLANTA, GEORGIA.

## COMPOSITION OF MATTER FOR LUBRICATING INTERNAL-COMBUSTION ENGINES.

1,369,678.

Specification of Letters Patent. Patented Feb. 22, 1921.

No Drawing.

Application filed September 5, 1918. Serial No. 252,733.

*To all whom it may concern:*

Be it known that I, LUTHER B. LOCKHART, a citizen of the United States, residing at Atlanta, in the county of Fulton and State 5 of Georgia, have invented certain new and useful Improvements in Composition of Matter for Lubricating Internal-Combustion Engines, of which the following is a specification.

10 My invention relates to a composition of matter for use in lubricating internal combustion engines, the same being adapted to be applied to the engines and parts thereof, internally and externally of the combustion 15 chambers.

An important object of the invention is to provide a lubricating composition of matter of the character described, that will have a specifically increased viscosity, when exposed to a high degree of heat, in the combustion chambers of the engine, and which will have a normal and not prohibitive viscosity, when functioning as applied to parts exteriorly of the combustion chamber.

20 In accordance with the preferred form of my invention, I employ heavy mineral oil, distilled or undistilled, or a heavy oil mixture. This heavy mineral oil is suitable to some extent, for the lubrication internally 25 and externally of internal combustion engines. With this heavy mineral oil, I thoroughly incorporate a small amount of a light mineral oil distillate, which is ordinarily too light for lubricating the parts of

30 an internal combustion engine, but heavier than light kerosene. The light oils employed are ordinarily of greater volatility than the light spindle oil. The light oil which gives the best result has about the volatility of 35 mineral seal, mineral sperm, or mineral colza oil. The light oils which I have found advantageous to employ are the heavy ends of kerosene, headlight oil, and heavy or high test illuminating oil.

40 I have found that satisfactory results are obtainable by employing from four to five per cent. by weight of the light oil with respect to the weight of the heavy oil but the invention is, of course, in no sense restricted to these proportions, as the same 45 may be widely varied as may be found advantageous. The resultant composition of matter has an approximately normal vis-

cosity, for lubricating the external parts of an internal combustion engine. 55

The following are specific examples of products employing my invention:

(A) Mineral oil of 600 Saybolt viscosity 96%, and headlight oil 4%.

(B) Mineral oil of 800 Saybolt viscosity 95%, and Leavy kerosene 5%.

(C) Mineral oil of 1200 Saybolt viscosity 94%, and mineral sperm oil 6%.

My composition of matter is therefore made up of viscous hydrocarbons, either distillates or undistilled residue, or a mixture of the same, with or without fixed oils, and a relatively small amount of specifically volatile hydrocarbons. As a result of this, the composition of matter has a decided deficiency or absence of hydrocarbons of intermediate boiling points. 70

In the use of my lubricating composition of matter, as applied to the exterior parts of an internal combustion engine, it has been 75 found that the composition of matter is of approximately normal viscosity, whereby lubrication proceeds normally, with very little volatilization of the light oil taking place. This small amount of volatilization 80 is largely due to the incorporation of the light oil with the heavy oil. Due to this incorporation, the light oil does not volatilize sufficiently from the composition of matter to form dangerous vapors exteriorly 85 of the combustion chamber, during prolonged exposure to normal heat of the lower cylinder walls.

Due to the normal viscosity of the lubricating composition of matter, only a normal 90 amount of the same will gain access to the interior of the internal combustion chamber, where it is instantly exposed to severe heat conditions. Under these conditions, the light oil volatilizes from the composition 95 of matter, also aiding in volatilizing off the lighter ends of the heavier oil. As a result of this, a heavier oil is left, applied to the walls of the cylinder to be consumed in the usual manner. This heavier oil has a higher 100 viscosity than the original composition of matter, and has a higher viscosity than an oil which can be directly and easily fed into the combustion chamber having a viscosity above 250 Saybolt at 100° F. This heavier 105 oil or oil residue produces and maintains a

film upon the wall of the cylinder, and this film can resist the action of heat to a greater extent. Further, the vaporization of the light oil produces a protective vapor film, 5 starting from the surface of the heavy oil film, which serves to protect the heavy oil film, to a considerable extent, from the action of hot gases, thereby prolonging its life. The prolongation of the life of the heavy oil 10 film, particularly during the firing stroke of the piston which is the most destructive stroke, is believed to produce important effects on the proper lubrication of the engine, during the succeeding stroke or strokes. In 15 many modern explosive engines, as for automobiles, etc., the oil film is exposed to the high heat of the explosion chamber for less than  $\frac{1}{10}$  of a second before the film can be renewed by the moving piston. It will be 20 readily seen that a slight prolongation of the life of the heavy oil film, will play an important part in lubricating the cylinder and piston, during the subsequent strokes.

It is to be understood that the form of my 25 invention herewith described is to be taken as a preferred example of the same and that various changes may be resorted to in the proportions in which the several ingredients are combined, and that known chemical 30 equivalents may be employed, without departing from the spirit of my invention, or the scope of the subjoined claims.

Having thus described my invention, I 35 claim:—

1. A composition of matter for lubricating internal combustion engines, consisting of a relatively large amount of heavy mineral oil, and a relatively small amount of light mineral oil incorporated therewith, 40 said light mineral oil having a high volatility but lower than the volatility of light kerosene, the light mineral oil being unsuitable for ordinary lubrication, the entire mass having a viscosity suitable for the external 45 lubrication of the engine, and the heavy mineral oil after the light mineral oil has been volatilized therefrom in whole or in part having a greater viscosity than the viscosity of the entire mass and being adapted for lubrication of the internal portions of the engine.

2. A composition of matter for lubricating internal combustion engines, consisting of a relatively large amount of heavy mineral oil, and a relatively small amount of light mineral oil incorporated therewith, said light mineral oil having a greater volatility than light spindle oil and a lesser volatility than light kerosene, the light mineral 60 oil being unsuitable for ordinary lubrication, the entire mass having a viscosity suitable for the external lubrication of the engine, and the heavy mineral oil after the light mineral has been volatilized therefrom 65 in whole or in part having a greater viscosity

than the viscosity of the entire mass and being adapted for the lubrication of the internal portions of the engine.

3. A composition of matter for lubricating internal combustion engines, consisting of approximately 19 parts of heavy mineral oil and approximately 1 part of a second oil having a volatility similar to mineral sperm oil, the second oil being unsuitable for ordinary lubrication, the entire mass having a viscosity suitable for the external lubrication of the engine, and the heavy mineral oil after the second oil has been volatilized therefrom in whole or in part having a greater viscosity than the viscosity of the entire mass and being adapted for the lubrication of the internal portions of the engine.

4. A composition of matter for lubricating internal combustion engines, consisting of a heavy oil, and approximately four per cent. by weight of mineral sperm oil, the entire mass having a viscosity suitable for the external lubrication of the engine, and the heavy mineral oil after the mineral sperm oil has been volatilized therefrom in whole or in part having a greater viscosity than the viscosity of the entire mass and being adapted for the lubrication of the internal portions of the engine.

5. A composition of matter for lubricating internal combustion engines, consisting of approximately 19 parts of heavy oil, and approximately 1 part of heavy illuminating oil, the entire mass having a viscosity suitable for the external lubrication of the engine, and the heavy mineral oil after the heavy illuminating oil has been volatilized therefrom in whole or in part having a greater viscosity than the viscosity of the entire mass and being adapted for the lubrication of the internal parts of the engine.

6. A composition of matter for lubricating internal combustion engines, consisting of a heavy oil and relatively small amount of light non-lubricating oil which is heavier than light kerosene whereby the composition has a substantial deficiency of hydrocarbons of intermediate boiling points.

7. A composition of matter for lubricating internal combustion engines consisting of a relatively large amount of heavy mineral oil having a viscosity higher than the viscosity of the composition to be produced and a relatively small amount of light mineral oils of a volatility between spindle oil and light kerosene the resultant composition having a viscosity substantially the same as the normal viscosity of lubricating oil.

In testimony whereof I affix my signature in presence of two witnesses.

LUTHER B. LOCKHART.

Witnesses:

T. B. HIGDON,  
W. E. DILLARD.